

# United States Patent Office

3,810,824

Patented May 14, 1974

1

3,810,824

## AQUEOUS ACID TIN-PLATING BATH

Donald Kearney Howard, Manchester, Brian Martin Thomas, Stockport, Cheshire, and Francis Popplewell, Manchester, England, and Dario Matossi, Pamplona, Spain, assignors to Ciba-Geigy Corporation, Ardsley, N.Y.

No Drawing. Original application Feb. 24, 1970, Ser. No. 13,766, now Patent No. 3,691,033. Divided and this application Aug. 10, 1972, Ser. No. 279,570. Claims priority, application Great Britain, Mar. 11, 1969, 12,804/69

Int. Cl. C23b 5/14, 5/46

U.S. CL. 204—54 R

9 Claims

### ABSTRACT OF THE DISCLOSURE

An aqueous acid tin-plating bath comprising a source of tin available for electro-plating, a source of hydrogen ions and an additive comprising from 0.0125% to 98.7% of 4,4'-di-(dimethylamino)-diphenylmethane and one or more tin-plating additives functionally active in an acidic tin-plating bath.

This application is a division of application Ser. No. 13,766, filed Feb. 24, 1970, now U.S. Pat. 3,691,033.

The present invention relates to new tin-plating additives and to tin-plating baths containing the additives.

It is known to use acidic tin-plating baths containing tin in the stannous form together with small amounts of organic additives. The incorporation of such organic additives into the tin-plating bath is made in order to increase the range of current density over which acceptable plating may be achieved. Examples of known organic tin-plating additives include condensed sulphonated phenol mixtures described and claimed in British Pat. No. 1,033,662.

However, by means of the incorporation of a tin-plating additive known for use in acidic baths or a mixture of such additives at their known working concentrations, acceptable plating is still only obtained within certain approximate limits of current density, for instance from about 60 amperes/square foot to about 450 amperes/square foot. Even at very high levels of addition, acceptable plating cannot be obtained at high current densities using known tin-plating additives alone or in admixture. In the specific case of 4,4'-di-(dimethylamino)-diphenylmethane, it is possible by the addition of very large amounts of this additive to achieve acceptable plating at very low current density but only at the expense of exceeding its solubility level in the bath and by recourse to the use of high voltages.

We have now discovered that a mixture of 4,4'-di-(dimethylamino)-diphenylmethane and one or more other tin-plating additives known to be functionally active in acidic tin-plating baths, when added at a similar level of concentration as conventional additives to an acidic tin-plating bath produces surprising synergistic effects resulting in satisfactory plating over a considerably wider range of current densities than can be obtained by the use of any of the additives singly or in other admixture.

Accordingly, the present invention provides a tin-plating additive comprising a proportion within the range of from 0.0125% to 98.7% by weight based on the total weight of the additive of 4,4'-di-(dimethylamino)-diphenylmethane and one or more tin-plating additives functionally active in an acidic tin-plating bath.

The present invention also provides a process in which a tin-plating additive is produced comprising admixing a proportion within the range of from 0.0125% to 98.7% by weight of 4,4'-di-(dimethylamino)-diphenylmethane

2

and one or more tin-plating additives functionally active in acidic tin-plating baths.

Although the 4,4'-di-(dimethylamino)-diphenylmethane may be employed successfully in high proportions in the tin-plating additive of the present invention, for optimal technical and economic advantage it is preferred not to exceed a proportion of 10% by weight. Thus, if more than 10% by weight of 4,4'-di-(dimethylamino)-diphenylmethane is present in the total additive, unacceptable levels of sludge-formation and/or of bath discoloration are observed in the tin-plating bath into which the tin-plating additive of the present invention is incorporated. A preferred range of proportions of 4,4'-di-(dimethylamino)-diphenylmethane in the total tin-plating additive is therefore from 0.0125% to 10% by weight, from 0.1% to 2.0% by weight being particularly preferred.

The second component of the tin-plating additive of the present invention may be selected from a range of additives known to be functionally active in conventional acidic tin-plating baths, especially the so-called "Ferrostan" bath, comprising an aqueous solution of stannous tin and phenol sulphonic acid. As examples of suitable additives there may be mentioned the sulphonated phenol additives produced according to the process described and claimed in British Pat. No. 1,033,662; the phenol/polyol condensation products described in co-pending British Pat. No. 1,221,688; sulphonated Bisphenol A-(2:2'-di-phenylolpropane) in acetic acid solution described in British Pat. No. 1,146,588; an additive consisting essentially of dihydroxydiphenyl sulphone under the trademark "Phenolene"; dihydroxydiphenyl sulphone as commercially available; and a commercially available sulphonated ethoxylated  $\alpha$ -naphthol additive.

Preferably the proportion of the second tin-plating additive is within the range of from 90% to 99.9875% by weight, more preferably within the range of from 98% to 99.9% by weight of the total tin-plating additive.

According to the present invention, there is also provided an acidic tin-plating bath comprising a source of tin available for electro-plating a source of hydrogen ions and an additive comprising a proportion within the range of from 0.012% to 98.7% by weight of 4,4'-di-(dimethylamino)-diphenylmethane and from 99.9875% to 1.3% by weight of one or more functionally-active tin-plating additives.

It is preferred to use stannous sulphate as the source of tin ions. The proportion of tin salt in the tin-plating bath is advantageously within the range of from 1.0% to 20% by weight, more preferably within the range of from 2.0% to 10% by weight, based on the total weight of the tin-plating bath.

The proportion of the tin-plating additive of the present invention in the tin-plating bath may be, for example, within the range of from 0.01% to 10% by weight, and preferably within the range of from 0.01% to 5% by weight, based on the total weight of the tin-plating bath.

In addition to the source of tin ions and the tin-plating additive of the present invention, the tin-plating bath desirably contains as the source of hydrogen ions, phenol sulphonic acid, the source of hydrogen ions preferably being present in a proportion within the range of from 0.1% to 20.0% by weight, more preferably within the range of from 0.5% to 10.0% by weight based on the total weight of the tin-plating bath.

The tin-plating additive of the present invention provides acceptable tin-plating from acidic tin-plating baths over a very wide range of current density. Moreover, the tin-plating additive of the present invention is compatible with other tin-plating bath components in all proportions which are conventionally employed for additives in acidic tin-plating baths.

The present invention is further illustrated by the following examples. Parts and percentages shown therein are by weight unless otherwise stated. Parts by weight bear the same relation to parts by volume as do kilograms to litres.

As a still further comparative aid, data is presented in Table 1 relating to the plating results achieved when only 4,4'-di-(dimethylamino)-diphenylmethane is employed as the tin-plating additive in the standard Hull test.

TABLE 1

| Example | Additives present in bath (grams/litre)                                            | Range of current density over which acceptable plating is achieved (amps/square foot) |                  |                                    | Current densities as corrected to allow for commercial plating line conditions |
|---------|------------------------------------------------------------------------------------|---------------------------------------------------------------------------------------|------------------|------------------------------------|--------------------------------------------------------------------------------|
|         |                                                                                    | Band position (cm.)                                                                   | Band width (cm.) | Actual hull cell current densities |                                                                                |
|         | Phenolene supra (condensation product of sulphonated o-cresol) (4.0).              | 3.3                                                                                   | 6.5              | 68 to 1.5.....                     | 450 to 64.                                                                     |
|         | Diphone V (sulphonated Bisphenol A derivative) (4.0)-----                          | 4.6                                                                                   | 4.6              | 45 to 2.0.....                     | 299 to 86.                                                                     |
|         | Dihydroxydiphenylsulphone (6.0)-----                                               | 4.3                                                                                   | 5.5              | 48 to 1.5.....                     | 330 to 64.                                                                     |
|         | Phenol/glucose condensation product (4.0).....                                     | 4.7                                                                                   | 5.1              | 45 to 1.5.....                     | 289 to 64.                                                                     |
|         | Diphone V (2.0) plus Phenolene Supra (2.0)-----                                    | 4.3                                                                                   | 5.5              | 48 to 1.5.....                     | 330 to 64.                                                                     |
|         | Phenolene supra (4.0) plus dihydroxydiphenylsulphone (1.0)-----                    | 4.1                                                                                   | 5.5              | 55 to 1.5.....                     | 350 to 72.                                                                     |
|         | TMADM (0.02)-----                                                                  | 5.5                                                                                   | 0.0              | Nil.....                           | Nil.                                                                           |
|         | TMADM (2.0)-----                                                                   | 4.0                                                                                   | 2.0              | 50 to 30.....                      | 350 to 260.                                                                    |
| 1-----  | Phenolene supra (4.0) plus TMADM (0.02)-----                                       | 0.2                                                                                   | 9.5              | >120 to 1.5.....                   | >700 to 68.                                                                    |
| 2-----  | Diphone V (4.0) plus TMADM (0.04)-----                                             | 0.4                                                                                   | 9.1              | >120 to 1.5.....                   | >700 to 76.                                                                    |
| 3-----  | Dihydroxydiphenylsulphone (6.0) plus TMADM (0.06)-----                             | 0.3                                                                                   | 9.7              | >120 to 1.2.....                   | >700 to 55.                                                                    |
| 4-----  | Phenol/glucose condensation product (2.0) plus TMADM (0.02)-----                   | 0.5                                                                                   | 9.0              | >120 to 1.5.....                   | >700 to 76.                                                                    |
| 5-----  | Phenolene supra (4.0) plus dihydroxydiphenylsulphone (1.0) plus TMADM (0.04).----- | 0.4                                                                                   | 9.1              | >120 to 1.7.....                   | >700 to 76.                                                                    |

## EXAMPLES 1-4

The acidic tin-plating bath solution having the following construction was made up.

| Parts by weight                                                                 |     |
|---------------------------------------------------------------------------------|-----|
| Electroplating grade of stannous sulphate (to British Standard 1468:1948) ----- | 55  |
| Phenol sulphonic acid -----                                                     | 30  |
| Water -----                                                                     | 915 |

To this solution was added 4,4'-di-(dimethylamino)-diphenylmethane in conjunction with the various tin-plating additive mixtures listed below in the respective amounts per litre as given in the following Table 1.

(a) The commercially-available product "Phenolene Supra" ("Phenolene" is a registered trademark) which is a condensation product derived from sulphonated o-cresol produced as described in British Pat. No. 1,033,662.

(b) The commercially-available product "Diphone V" which is believed to be a sulphonated Bisphenol A derivative and is also believed to be described and claimed in British Pat. No. 1,146,588.

(c) The commercially-available product "Phenolene" which consists substantially of dihydroxydiphenylsulphone ("Phenolene" is a registered trademark).

(d) A phenol/glycose condensation product described and claimed in our copending British Pat. No. 1,221,688.

250 millilitres of each of the respective solutions were placed in turn in a standard 350 millilitres Hull cell (W. Nohse, the "Hull Cell" published R. Draper Limited, 1966) and plating was carried out at 3.0 amps at 50° C. for one minute. The results obtained are summarized in Table 1.

For the purpose of comparison, data are also included in Table 1 relating to the use of the additives listed under headings (a) to (d) alone, that is, in the absence of 4,4'-di-(dimethylamino)-diphenylmethane (TMADM) in Hull cell tests under the standard conditions described in the previous paragraph.

As a further comparative aid, data is given in Table 1 relating to the plating results achieved when, as the tin-plating additive, a mixture of equal parts by weight of additives (a) and (b) listed above is employed in the standard Hull test.

## What we claim is:

1. An aqueous acidic tin-plating bath comprising a source of tin available for electroplating, a source of hydrogen ions and from 0.01 to 10% by weight of the tin-plating bath of an additive comprising from 0.0125% to 98.7% by weight of 4,4'-di-(dimethylamino)-diphenylmethane and from 99.9875 to 1.3% by weight of one or more tin plating additives selected from sulphonated phenol additives produced by sulphonating phenol and/or cresol with oleum containing 60% to 66% by weight of sulphur trioxide and thereafter heating the resulting sulphonated product for at least one hour without adding further phenol, at a subatmospheric pressure of from 5 to 25 millimeters of mercury and at a temperature in the range of from 120° C. to 190° C.; the phenol polyol condensation products produced by reacting phenol and an aliphatic polyol containing from 2 to 8 hydroxyl groups per molecule in a 1:1 to 10:1 molar proportions respectfully the condensation reaction being carried out at a temperature of from 50° C. to 250° C.; sulphonated Bisphenol A-(2,2'-di-p-phenylolpropane) in acetic acid solution; an additive consisting essentially of dihydroxydiphenylsulphone and sulphonated ethoxylated  $\alpha$ -naphthol.
2. A tin-plating bath as claimed in claim 1 wherein the proportion of tin salt in the tin-plating bath is within the range of from 1.0% to 20% by weight based on the total weight of the bath.
3. A tin-plating bath as claimed in claim 2 wherein the proportion of salt in the tin-plating bath is within the range of from 2.0% to 10% by weight based on the total weight of the bath.
4. A tin-plating bath as claimed in claim 3 wherein the proportion of the tin-plating additive is within the range of from 0.01% to 5% by weight based on the total weight of the tin-plating bath.
5. A tin-plating bath as claimed in claim 1 wherein the proportion of the source of hydrogen ions is within the range of from 0.1% to 20% by weight based on the total weight of the bath.
6. A tin-plating bath as claimed in claim 5 wherein the proportion of the source of hydrogen ions is within the range of from 0.5% to 10% by weight based on the total weight of the bath.

7. A tin-plating bath as claimed in claim 1 wherein stannous sulphate is employed as the source of tin ions.
8. A tin-plating bath as claimed in claim 1 wherein the source of hydrogen ions is phenol sulphonic acid.
9. A method in which tin-plate is produced comprising electroplating onto a substrate using a tin-plating bath claimed in claim 1.

## References Cited

## UNITED STATES PATENTS

|           |        |              |          |
|-----------|--------|--------------|----------|
| 2,846,381 | 8/1958 | Frick et al. | 204-54 R |
| 3,515,653 | 6/1970 | Sykes        | 204-54 R |

GERALD L. KAPLAN, Primary Examiner